

## UNITED STATES PATENT OFFICE

2,380,711

## CHROMIUM-FREE AIR-HARDENING ALLOY STEELS AND ARTICLES OF MANUFACTURE PRODUCED THEREFROM

Enrique G. Touceda, Loudonville, and Ralph P. De Vries, Menands, N. Y., assignors to Allegheny Ludlum Steel Corporation, a corporation of Pennsylvania

No Drawing. Application July 28, 1942,  
Serial No. 452,638

10 Claims. (Cl. 75—125)

Our present invention relates to air-hardening alloy steels which are useful both in the cast and in the wrought condition for the production of tools, dies and structural members and which are characterized by the fact that they contain a small amount of beryllium but no chromium.

Conventional air-hardening steels containing chromium are expensive to harden and are definitely restricted as to the degree of hardness which can be imparted thereto. Hardening is carried out from temperatures in the range of 1800-1900° F. and considerable difficulty is encountered in obtaining hardness values as high as 600 Brinell. Care must also be taken to correlate properly the carbon and chromium contents in order to minimize or avoid undue brittleness, loss of toughness, decrease in hardenability and poor fluidity.

Air-hardening steels of the Mushet type contain a substantial amount of tungsten and sometimes a small amount of chromium and are likewise expensive and rather difficult to produce. While both types of air-hardening steels are commercially employed they are far from ideal, with the result that the industry is still seeking improved compositions which are more versatile in their applications.

One of the objects of our present invention is to produce alloy steels which are air-hardening and yet which contain no chromium or tungsten, which are easier and less expensive to harden and which can readily be hardened to high hardness values from relatively low temperatures.

Another object of our invention is to produce a beryllium-containing chromium-free air-hardening alloy steel which has new and useful properties and characteristics and which in particular is capable of readily acquiring a hardness value of at least 600 Brinell and 60 Cone Rockwell by air cooling after heat treating to the abnormally low temperatures of 1450-1550° F.

A further object of our invention resides in producing new and useful alloy steels of substan-

tially the following composition: carbon, .05-2.50%; silicon, .50-2.50%; manganese, .75-3.25%; molybdenum, 25-2.50%; copper, .35-2.00%; and beryllium, .03-30%, the balance being substantially all iron except for the usual impurities in normal amounts.

A still further object of our invention is to produce beryllium-containing alloy steels as herein-after defined in which the formation of graphite in castings and forgings can be controlled.

A still further object of our invention is to provide air-hardening steels containing beryllium and copper and which can be cast to shape and size with good fluidity.

15 Other and further objects and advantages will be understood by those skilled in this art or will be apparent or pointed out hereinafter.

Our invention is predicated upon the discovery that alloy steels with unusually good hardening properties can be produced without chromium or tungsten by incorporating beryllium therein especially in conjunction with copper.

We have discovered that even extremely small amounts of beryllium in the presence of copper and in combination with the other elements specified, not only renders such steels air-hardening but they can be hardened to high values of hardness above 600 Brinell and 60 Cone Rockwell. Even a few hundredths of a per cent of beryllium endow these alloy steels with the desired properties and in addition make possible a substantial decrease in the cost of hardening because hardening can be effected from abnormally low temperatures of about 1450-1550° F. in direct contrast with prior steels which must be hardened from a temperature of 1800-1900° F. The elimination of chromium has advantages which will be appreciated by the metallurgist and in addition steels containing beryllium and copper are far superior to chromium and tungsten steels for many purposes.

Our new alloy steels consist of, in addition to iron and the usual impurities in normal amounts,

about .05-2.50% carbon, about .50-2.50% silicon, about .75-3.25% manganese, about 25-2.50% molybdenum, about .35-2.00% copper, and about .03-.30% beryllium.

Illustrative examples of compositions responding to our present invention and a few other compositions included for comparative purposes are set forth in Table I, which follows:

same amount of copper as T-218. It is further noteworthy that the beryllium content of composition T-215 is only .04% and that the amounts of the other elements are comparable. The significance of this will be more fully appreciated from composition T-241 which in a cast piece having a cross section about three times as great as composition T-215 has practically undimin-

Table I

| Melt No. | C    | Si   | Mn   | Mo   | Cu   | Be   | As annealed |    |      | As forged       |     |        | Size cross sec. | 1450° F.   | Air file | Size cross sec. | As cast |    |          | Mag. change point F. |  |  |  |  |  |
|----------|------|------|------|------|------|------|-------------|----|------|-----------------|-----|--------|-----------------|------------|----------|-----------------|---------|----|----------|----------------------|--|--|--|--|--|
|          |      |      |      |      |      |      | Br          | RC | File | Br              | RC  | File   |                 | 1450° F.   |          |                 | Br      | RC | 1450° F. |                      |  |  |  |  |  |
|          |      |      |      |      |      |      |             |    |      |                 |     |        |                 |            |          |                 |         |    |          |                      |  |  |  |  |  |
| T-203    | 1.27 | 1.74 | 2.20 | .90  | 1.30 | .04  | 265         | 25 | F    | 1" sq.          | 627 | 63     | Hard            | 3 1/2 x 5" | 601      | 62              | Hard    | do | 260      |                      |  |  |  |  |  |
| T-204    | 1.38 | 1.42 | 1.90 | .98  | 1.30 | .04  | 241         | 27 | F    | 2 1/2" square.  | 601 | 57     | Hard            | 3 1/2 x 5" | 601      | 59              | Soft    | do | 260      | 1,200                |  |  |  |  |  |
| T-205    | 1.29 | 1.56 | 1.91 | 1.26 | —    | —    | 277         | 25 | F    | 2 1/2" square.  | 627 | 62 1/2 | Hard            | 3 1/2 x 5" | 321      | 24              | Hard    | do | 600      |                      |  |  |  |  |  |
| T-214    | 1.25 | 1.95 | 2.19 | 1.06 | —    | —    | 260         | 28 | F    | 1 1/2" RD       | 627 | 61     | Hard            | 2 1/2 x 2" | 578      | 50              | Hard    | do | 300      |                      |  |  |  |  |  |
| T-215    | 1.26 | 1.67 | 1.96 | 1.52 | 1.28 | .04  | 277         | 29 | F    | 1 1/2" RD       | 601 | 61     | do              | 3 x 2 1/2" | 653      | 62              | do      | do | 300      |                      |  |  |  |  |  |
| T-218    | 1.11 | .82  | 1.57 | 1.90 | 1.30 | —    | 321         | 22 | F    | 2 1/2" x 2 1/2" | 601 | 62     | Soft            | 3 x 2 1/2" | 601      | 60              | Soft    | do | 450      |                      |  |  |  |  |  |
| T-219    | 1.12 | .80  | 1.54 | 1.86 | —    | —    | 265         | 29 | F    | 2 1/2" x 2 1/2" | 603 | 41     | Soft            | 3 x 2 1/2" | 241      | 38              | do      | do | 300      |                      |  |  |  |  |  |
| T-241    | 1.41 | 1.88 | 2.92 | 1.54 | 1.28 | .04  | 321         | 22 | F    | 5 x 4 1/2"      | 653 | 61     | Hard            | 5 x 4 1/2" | 653      | 61              | Hard    | do | 1,100    |                      |  |  |  |  |  |
| 50544    | 1.39 | 1.71 | 2.58 | 2.03 | 1.45 | .088 | —           | —  | —    | 4 x 4"          | 652 | 63     | Hard            | —          | —        | —               | —       | —  | —        | —                    |  |  |  |  |  |

NOTES.—(a) "F"=soft. (b) Magnetic change point—the magnetic changes noted on cooling from the hardening temperature indicated.

This table illustrates the hardness values that can be secured by hardening from a temperature of 1450° F. followed by air cooling both in the as forged and in the as cast conditions. These compositions which contain neither copper nor beryllium are in general of less hardness than is required for present purposes but in evaluating hardness values due regard must be given to the dimensions of the piece in question as will be more fully appreciated from our co-pending application, Serial Number 452,637, filed July 28, 1942. In that application we have pointed out that, other things being equal, hardness values are inversely proportional to the mass of metal involved, particularly the cross-sectional area of the piece undergoing hardening. Therefore, merely because a given procedure will produce desirable hardening characteristics in a piece of one size does not signify that the same hardness characteristics will result when all the conditions are the same except that the size of the treated piece is larger. These statements apply particularly to steel T-214 which in a piece 1 1/2" round (corresponding to a cross-sectional area of 1.76 sq. in.) can be hardened to 627 Brinell and 61 Cone Rockwell but in the cast state with dimensions of 2" x 2 1/2" (corresponding to a cross-sectional area of 5 sq. in.) hardens to a considerably less extent, viz., only to 578 Brinell and 59 Cone Rockwell. In still larger sizes it does not even approach the required hardness of 600 Brinell and 60 Cone Rockwell either in the as cast or in the as rolled condition.

Contrasted with this, steel T-218 (Table I) which contains 1.3% of copper but no beryllium shows good hardness characteristics as forged to a piece 2" x 2 1/2" (which corresponds to a cross-sectional area of 5 sq. in.) and still shows nearly the same hardness characteristics in a casting having the dimensions of 2 1/2" x 3" (which corresponds to a cross-sectional area of 7 1/2 sq. in.). However, upon comparing the hardness values of composition T-218 with composition T-215 it will be found that the latter containing both copper and beryllium has definitely superior hardness values even though it contains approximately the

30 ished hardness values. Composition 50544 is likewise notable in that a forged section more than three times as great as composition T-218 and more than nine (9) times as great as composition T-215 shows the highest Brinell hardness value and a Cone Rockwell hardness equal to the best obtained for any composition and size,—even the 1" forged section of composition T-203 which has excellent hardness characteristics.

35 As will be apparent from the ranges set forth above, the carbon content of our new compositions may range from a minimum of about .05% to a maximum of about 2.5% and our compositions present no difficulty in forging or rolling throughout this carbon range except that for values of 1.50-2.25% of carbon forging and rolling are somewhat less readily effected. The various ranges of compositions do, however, have marked differences with reference to size limitations of hardening and when the silicon content is lowered below .75% hardening is materially less effective than in those compositions containing more than .75% of silicon. These facts make it necessary to exercise considerable caution in evaluating the results obtained because steels containing an amount of silicon in the lower portion of the range specified can still be hardened from a low temperature. The higher silicon steels in conjunction with the higher carbon contents of the order of 1-1.5% contain more graphite than like compositions with lower silicon and carbon percentages but neither the particular amount of graphite present nor the presence or absence of graphite prevents effective hardening.

40 45 50 55 60 65 70 75 80 85 90 95 With a carbon content in the upper portion of the specified range, i. e., from approximately 1.50-2.25% of carbon, our steels are especially useful in the as cast condition. Such steels are usually air-hardenable up to sections as large as those which are air-hardenable when they contain carbon in the range of approximately 1.25-1.50%. Those cast steels containing approximately 1.50-2.25% of carbon have an advantage in that they are more easily machinable

than steels containing carbon within the range of approximately 1.25-1.50%. This is due to the fact that the hardness values of the former are somewhat lower than those of the latter after annealing.

The occurrence of graphite in the manufacture of air-hardening steels containing the above indicated amounts of silicon from a cast ingot to a finished forged or rolled bar, or during the manufacture of any particular casting to the finished forging, is primarily a function of the mass of metal involved in the particular operation. Our investigations showed the presence of free graphite in small masses of metal and

of such composition that they can be hardened from low temperatures and which when so hardened, are characterized by physical properties suitable for use as tool and die steels.

In some instances deliberate production of graphite is desired for purposes other than special tool and die steels and we have found that graphite in well-formed and well-distributed nodules can readily be produced in such articles as thin-walled cylinders and the like from those steels embraced within our present invention which contain approximately 1-1.5% of carbon. Reference is had to Table II which follows:

Table II

| Melt # | C    | Si   | Mn   | Mo   | Cu   | Ni    | Be    | As annealed 5 hr. 1640° F. |       | File  | F.° heat treatment | Rockwell Cone | Brinell | Size        |
|--------|------|------|------|------|------|-------|-------|----------------------------|-------|-------|--------------------|---------------|---------|-------------|
|        |      |      |      |      |      |       |       | Br                         | RC    |       |                    |               |         |             |
| T-196  | 1.25 | 2.00 | 1.50 | 1.25 | 1.50 | ----- | .05   | 255                        | 25    | Soft  | -----              | -----         | 555     | 1" x 3"     |
| T-196  | 1.39 | 2.00 | 1.70 | 1.26 | 1.56 | ----- | ----- | 262                        | 27    | Soft  | 1,450/1 hr. air    | 56            | 682     | 3/4 x 3"    |
| T-197  | 1.25 | 1.50 | 1.50 | 1.75 | 1.25 | ----- | .04   | -----                      | ----- | ----- | 1,450/2 hr. air    | 63            | 653     | 2" x 1 1/2" |
| T-197  | 1.39 | 1.48 | 1.64 | 1.90 | 1.27 | ----- | ----- | 223                        | 19    | Soft  | 1,450/2 hr. air    | 60            | 601     | 2" x 1 1/2" |
| T-198  | 1.25 | 2.00 | 1.25 | 1.25 | 1.50 | 0.75  | .05   | -----                      | ----- | ----- | 1,400/2 hr. air    | 58            | 555     | 2 sq. x 2"  |
| T-198  | 1.35 | 1.84 | 1.38 | 1.26 | 1.54 | .87   | ----- | 363                        | 39    | Soft  | 1,400/2 hr. air    | -----         | -----   | -----       |
| T-199  | 1.10 | 2.20 | 3.25 | .80  | 1.50 | ----- | .05   | -----                      | ----- | ----- | -----              | -----         | -----   | -----       |
| T-199  | 1.18 | 1.95 | 3.44 | 1.06 | 1.50 | ----- | ----- | -----                      | ----- | ----- | -----              | -----         | -----   | -----       |

the substantial absence of graphite in larger masses of metal. As an illustration, we melted 600 pounds of steel having the following composition: carbon, 1.39%; silicon, 1.71%; manganese, 2.58%; molybdenum, 2.03%; copper, 1.45% and beryllium, .09%, it being understood that the balance of the steel was iron and the usual impurities in normal amounts. This 600 pound heat was cast into an ingot 8 inches square. Three portions of that ingot were forged to billets which were respectively 6 inches square, 4 inches square and 2 inches square, and in producing these billets the identical heat treatment was given to the three different ingot portions and after forging the three billets were given identical annealing operations. Examination of these billets showed the presence of free graphite in the 2 inch square billet but the 4 inch square and 6 inch square billets showed practically no

Such steels can be cast and forged and subsequently hardened to the hardness of tool steel (substantially to 600 Brinell or more) and they may contain graphite. The presence of graphite can be insured, as will be appreciated from what has preceded, either by making the initial casting of comparatively small size or section or by forging an initially large casting or a portion of an initially large casting into such size that graphite is formed easily during the forging and subsequent annealing operations. Thus, in accordance with our invention and in connection with compositions having 1-1.5% of carbon, as exemplified by Table II, the production of graphite is easily controlled and those forgeable graphite-containing steels may be utilized in an unhardened or semi-hardened state if preferred or desired.

Table III, which follows, illustrates compositions with a carbon content near the upper portion of the indicated range:

Table III

| Melt # | C    | Si   | Mn   | Cu   | Mo    | Be  | As annealed chill cast Rockwell | Heat treat- ment | Size          | Cone Rockwell | File  |
|--------|------|------|------|------|-------|-----|---------------------------------|------------------|---------------|---------------|-------|
|        |      |      |      |      |       |     |                                 | 99.5B            | 1,400° F. air | 5/8" rd.      | 60    |
| T-53   | 1.76 | 1.79 | 1.38 | .85  | ----- | .10 | 99.5B                           | 1,400° F. air    | 5/8" rd.      | 60            | Hard. |
| T-54   | 1.87 | 1.13 | 1.64 | .85  | ----- | .10 | 21.5C                           | do               | do            | 61            | Do.   |
| T-55   | 2.00 | 1.00 | 1.50 | 1.00 | 0.75  | .10 | 31C                             | do               | do            | 64            | Do.   |

free graphite. The cycle of heating preliminary to the forging and annealing after forging were of such extended duration that the absence, or substantial absence of graphite could not possibly be due to inadequate heating. It is thus clear that the size of the initial casting and the size of the forging produced therefrom has a controlling effect upon the production of free graphite in the low temperature air-hardening steels responding to our present invention. For most tool and die purposes the presence of graphite is not an essential part of our invention and its presence does not prevent the accomplishment of the desired hardening effect. Our invention thus includes the production of steels

60 The designated steels are particularly useful for castings employing a relatively large amount of carbon such as cast cylinders and the like, but these high carbon steels have only a relatively limited application to tool steel purposes. These steels still harden well in small sizes from temperatures as low as 1400-1500° F. and at slightly higher temperatures a somewhat greater degree of hardness can be secured. The steels of Table III, however, exemplify a distinct class of steels which can be easily machined in the cast and annealed condition and in which the order of machinability is that of a good grade of gray cast iron.

Reference is next had to Table IV, which follows:

Table IV

| Heat # | C    | Mn   | Si   | Cu   | Mo   | Be  | Size                | Annealed 1700° F. (cool 30° / hr. 900° F. Brinell) | 1450° F. 6 hr. air Brinell | 1525° F. 6 hr. air Brinell |
|--------|------|------|------|------|------|-----|---------------------|----------------------------------------------------|----------------------------|----------------------------|
| 202    | 1.03 | 2.08 | 1.57 | 1.26 | 2.60 | .06 | 5" rd. x 5" long... | 302                                                | 678                        | 601                        |
| 203    | 1.43 | 1.36 | 1.36 | 1.26 | 2.52 | .06 | do                  | 302                                                | 578                        | 601                        |
| 204    | 1.76 | 2.08 | 1.41 | 1.28 | 2.54 | .06 | do                  | 285                                                | 578                        | 578                        |
| 205    | 1.48 | 2.08 | 1.48 | 1.28 | 2.62 | do  | do                  | 293                                                | 352                        | 363                        |

In this table we show the analyses and hardening characteristics of four different heats of steel cast into rounds 5 inches in diameter and 5 inches long. From this table it can be observed that heat #205 containing neither copper nor beryllium hardens to an extent only little more than half of the hardness value of heats #202, #203 and #204, even though the balance of the compositions was substantially identical. Thus, compositions such as those set forth and containing both copper and beryllium can be easily hardened to high hardness values of substantially 600 Brinell or more in direct contrast to a similar composition but without copper and beryllium.

In our co-pending applications, Serial No. 452,636, filed July 28, 1942, and Serial No. 452,639, filed on July 28, 1942, we have described chromium - containing air - hardening steels which can be cast to ultimate shape and dimensions with good fluidity. The same thing is true of our present compositions even though they contain no chromium and this, it will be appreciated, is a worthwhile advantage. While we have shown that the higher carbon steels can be air-hardened from unusually low temperatures around 1450° F., steels with lower carbon contents and containing percentages of elements at or near the lower portions of the ranges set forth have been found to be very useful steels both in the form of castings and in the wrought condition as obtained by forging or rolling and this results chiefly from the fact that the exceptional fluidity during casting produces castings of unusually good physical properties subsequent to appropriate heat treatments. These steels can only be air-hardened when in the smallest sizes or sections but depending upon the amount of hardness desired they can be quenched in oil or in water to produce excellent physical strength and elongation. A typical set of such cast steels and the physical properties thereof are set forth in Table V. These steels can be quenched, irrespective of whether or not they have had a preliminary subcritical anneal, to produce cast parts having adequate strength coupled with high ductility:

Having described our invention, what we claim as new and desire to secure as Letters Patent are:

1. A tool, die and structural steel consisting of the following elements in substantially the following amounts: .05-2.50% of carbon, .50-2.50% of silicon, .75-3.25% of manganese, .25-2.50% of molybdenum, .35-2.00% of copper and .03-30% of beryllium, the balance being substantially all iron except the usual impurities in common amounts.

2. An alloy steel consisting of about 1.3% carbon, about 1.5% silicon, about 2% manganese, about 1% molybdenum, about 1.3% copper, and a small amount of beryllium less than 1%, said alloy steel being characterized by the fact that it can be hardened from a temperature of about 1450° F. to a Brinell value of at least 600 and a Rockwell Cone value of at least 60 in both the as cast and the as forged condition.

3. A chromium-free air-hardening tool and die steel consisting of about .05-2.50% of carbon, about .50-2.50% of silicon, about .75-3.25% of manganese, about .25-2.50% of molybdenum, .35-2.00% of copper, and about .03-30% of beryllium, with the balance substantially all iron except for the usual impurities in normal amounts.

4. A chromium and tungsten-free air-hardening tool and die steel consisting of about .05-2.50% of carbon, about .50-2.50% of silicon, about .75-3.25% of manganese, about .25-2.50% of molybdenum, about .35-2.00% of copper, and about .03-30% of beryllium, with the balance substantially all iron except for the usual impurities in normal amounts, said steel being characterized by the fact that forgings and castings can be produced therefrom in which the graphite content can be readily controlled.

5. An article of manufacture composed of an alloy steel having the composition defined by claim 3 and containing graphite, the graphite content being substantially uniformly distributed throughout said article in the form of well-defined nodules.

6. An alloy steel capable of being hardened

Table V.

| Melt # | C   | Si   | Mn   | Mo   | Cu   | Be  | State                                       | Brinell | Yield point, p. s. i. | Tensile strength, p. s. i. | Elong. percent in 2" | Red. area, percent |
|--------|-----|------|------|------|------|-----|---------------------------------------------|---------|-----------------------|----------------------------|----------------------|--------------------|
| 424-A  | .27 | 1.50 | 1.00 | 1.00 | 1.00 | .10 | As cast 1,450° F. Oil-drawn. 750° F. air.   | -----   | 95,000                | 192,500                    | 8.0                  | 11.2               |
| 424-A  | .27 | 1.50 | 1.00 | 1.00 | 1.00 | .10 | As cast 1,400° F. 1/4 hr. oil.              | 444     | 68,000                | 219,000                    | 4.5                  | 7.8                |
| 425-A  | .29 | 1.00 | 1.50 | 1.00 | 1.00 | .10 | As cast 1,400° F. 1/4 hr. oil.              | 415     | 116,000               | 216,500                    | 3.0                  | 4.4                |
| 425-A  | .29 | 1.00 | 1.50 | 1.00 | 1.00 | .10 | As cast 1,750° F. Oil-drawn. 570° F. air.   | -----   | 100,000               | 226,000                    | 3.5                  | 10.3               |
| 426-A  | .27 | .75  | 1.50 | 1.00 | 1.00 | .10 | As cast 1,750° F. Oil-drawn. 1,375° F. air. | -----   | 72,700                | 196,950                    | 2.0                  | 4.4                |

The foregoing is illustrative and not limitative and various additions, omissions, substitutions and modifications may be made therein without departing from the spirit and scope of our invention as defined by the appended claims.

to at least about 600 Brinell and 60 Cone Rockwell from a temperature of from about 1450° F. to 1550° F., and which in addition to iron and the usual impurities consists of from about 1.00% to about 1.50% carbon, from about .75% to about

2.50% silicon, from about .75% to about 3.25% manganese, from about .80% to about 2.50% molybdenum, from about .35% to about 2.00% copper and from about .03% to about .30% beryllium.

7. An alloy steel which in addition to iron and the usual impurities in common amounts consists of from about 1.50% to about 2.25% carbon, from about 1.00% to about 2.50% silicon, from about 1.50% to about 3.25% manganese, from about 1.50% to about 2.50% molybdenum, from about 1.20% to about 1.50% copper and from about .03% to about .30% beryllium.

8. An alloy steel which in addition to iron and the usual impurities in common amounts consists of from about .25% to about .30% carbon, from about 1.00% to about 1.50% silicon, from about 1.00% to about 1.50% manganese, approximately 1.00% molybdenum, approximately 1.00% copper and approximately .10% beryllium.

9. A ferrous alloy containing a substantially

uniform distribution of graphite comprising from about 1.00% to about 1.50% carbon, from about 1.50% to about 2.50% silicon, from about 1.50% to about 3.25% manganese, from about 0.25% to about 2.50% molybdenum, from about 1.25% to about 2.00% copper and from about 0.03% to about 0.3% beryllium, with the remainder substantially all iron.

10. A chromium-free, air-hardening tool and die steel containing from about 0.27% to about 2.50% carbon, from about 0.75% to about 2.50% silicon, from about 1.25% to about 3.25% manganese, from about 0.75% to about 2.25% molybdenum, from about 0.80% to about 2.00% copper and from about 0.03% to about 0.30% beryllium, with the remainder substantially all iron characterized by the fact that it can be hardened to a value of at least 800 Brinell from temperatures of from about 1480° F. to about 1550° F.

20 ENRIQUE G. TOUCEDA.  
15 RALPH P. DE VRIES.